

# UNITED STATES PATENT OFFICE.

FOSTER MILLIKEN, OF LAWRENCE, NEW YORK, ASSIGNOR TO FOSTER MILLIKEN,  
S. FULLERTON WEAVER, AND JAMES M. REPLIER, TRUSTEES.

## ALLOY.

1,338,518.

Specification of Letters Patent. Patented Apr. 27, 1920.

No Drawing. Original application filed August 29, 1918, Serial No. 251,941. Divided and this application filed December 11, 1918. Serial No. 266,328.

To all whom it may concern:

Be it known that I, FOSTER MILLIKEN, a citizen of the United States, and a resident of Lawrence, in the county of Nassau and 5 State of New York, have invented a new and Improved Alloy, of which the following is a full, clear, and exact description, this being a division of the application, Serial No. 251,941, filed by me on August 29, 1918. 10 The object of the invention is to provide a new and improved alloy characterized by having a high acid resisting quality, an increased density, an exceedingly close and fine grain, great tensile strength, increased 15 elasticity, and electrical resistance.

The alloy is formed of copper, nickel, iron and zinc under the influence of chromium.

In carrying out the invention use is made of copper, 50 to 60 per cent.; nickel, 26 to 20 34 per cent.; iron, 4 to 8 per cent.; zinc, 7 to 11 per cent.; and chromium, .25 to 5 per cent.

The metal in each case consists of one hundred ounces of the four metals and the 25 percentage of chromium is then added extra. A large percentage of chromium after the latter has done the work of purifying the alloy, passes off in the slag, and the remaining small percentage of chromium 30 forms a component part of the alloy. Adding the chromium to the previously formed alloy of copper, nickel, iron and zinc permits of using a comparatively small amount of chromium for the purpose of purifying 35 the alloy.

It is understood that the addition of chromium has the double function of purifying the copper, nickel, iron and zinc and of adding a valuable ingredient to the alloy 40 as follows:

Specimens of the alloy tested for three

months in the acid test disclosed, with the alloy formed under the influence of chromium, a loss of .0079 to .0117 per square inch, and hence it is manifest that an alloy of 45 the character specified has high acid resisting properties. It has also been found that an alloy produced under the influence of chromium has increased density and the grain is closer and finer and resistance to 50 corrosion is increased.

It is expressly understood that the de-oxidizing agent removes any oxidized portions that may have formed on any one of the metals forming the alloy and hence no 55 cavities, fissures, recesses or the like and incident to oxidation are formed in the alloy. The alloy is thus compacted and its elastic limit and tensile strength are considerably increased relative to any alloy 60 formed of the same metals without the influence of the deoxidizing agent. It is well known that when a metal is deoxidized and is free of cavities and the like its electrical 65 resistance is increased and this is expressly the case in the present alloy. It has been found that the alloy as described and having the addition of a trace of chromium has a tensile strength of approximately 89,600 lbs. with an elastic limit of over 60% of the 70 tensile strength.

Having thus described my invention, I claim as new and desire to secure by Letters Patent:—

An alloy consisting of the following ingredients in about the following proportions, copper 50 to 60 per cent., nickel 26 to 34 per cent., iron 4 to 8 per cent., zinc 7 to 11 per cent., the said copper, nickel, iron and zinc being in a deoxidized state, and chromium. 75 80

FOSTER MILLIKEN.